

C. GERARD.

PROCESS FOR THE SOLIDIFICATION OF PETROLEUM.  
APPLICATION FILED MAR. 22, 1912.

1,085,119.

Patented Jan. 27, 1914.



Witnesses:

Walter M. Chapin  
Ida M. Patterson.

Inventor  
Charles Gerard  
By  
Resubmitted by  
John

# UNITED STATES PATENT OFFICE.

CHARLES GERARD, OF BRUSSELS, BELGIUM.

## PROCESS FOR THE SOLIDIFICATION OF PETROLEUM.

1,085,119.

Specification of Letters Patent. Patented Jan. 27, 1914.

Application filed March 22, 1912. Serial No. 685,616.

To all whom it may concern:

Be it known that I, CHARLES GERARD, a subject of the King of Belgium, residing at Brussels, in the Kingdom of Belgium, have invented new and useful Improvements in Processes for the Solidification of Petroleum, of which the following is a specification.

This invention relates to a process for the solidification of crude petroleum and other hydrocarbons for the purpose of enabling them to be used directly as a fuel or as an agglomerating product in the manufacture of agglomerates having suitable solid combustible materials for a base. This process is based, like other known processes, upon the conversion of petroleum into a rather thick starchy paste by the addition of fecula or other equivalent products.

The object of the invention is, chiefly, to avoid the objections which are inherent to the processes hitherto employed for the solidification of petroleum, which processes are generally based upon the saponification, resinification, or the treatment of petroleum with starch. These objections are well known in trade and principally arise through the petroleum not being sufficiently enveloped by the material which has served to form a starchy paste therewith and thereby runs when put in the fire.

With the object of remedying this defect, my invention is mainly based upon the use, in combination with petroleum and with fecula serving to form a starchy paste therewith, of a certain quantity of hot water the function of which may be explained as follows:

When petroleum is formed into a starchy paste by mixing it with the residues of fatty bodies or of fecula according to the ordinary methods it has been found that the mixture becomes consistent upon cooling and the petroleum does not run. As soon, however, as the fuel is put in the fire, the petroleum liquefies and runs into the ash pit of the furnace. On the contrary, if, at the moment of mixing the petroleum with fecula a certain quantity of hot water brought to boiling point is interposed, it will be found that under the action of the boiling water a swelling of the grains of the fecula will be produced and these can then at once absorb the water and the petroleum. After cooling the starchy paste thickens and neither the heating in the

mixer used for the manufacture of agglomerated fuel nor the heat of the furnace will reliquify the petroleum, that is to say, expel it from the grains of fecula by which it is, so to speak, enveloped. The petroleum then burns in a perfect manner and without running.

In carrying out the invention I proceed as follows: The crude petroleum to be treated is placed in a steam-heated vessel and is therein brought to a suitable temperature, for example, to about 25° to 30° C. A second vessel, heated by means of steam or by a fire, contains water which is brought to boiling point and maintained at boiling temperature by suitable heating. A third vessel contains the fecula used in the formation of the starchy paste. The employment of these three vessels is combined with the use of a mixing apparatus provided with an agitator. Into this mixing apparatus is poured a certain quantity of fecula coming from the third vessel, above mentioned and, through suitable pipes connecting the mixer with the two first vessels a certain quantity of petroleum and boiling water are allowed to flow into the mixer, the agitator of which is in motion. Fecula, petroleum and boiling water are afterward successively added in varying proportions according to the result which it is desired to obtain. When the mixture is sufficiently intimate it is removed from the mixer and a more or less thick product is thus obtained which solidifies upon cooling. This product can be employed directly as fuel or can be mixed by any known process with suitable solid materials so as to form agglomerated fuel. Afterward stearic, palmitic oleic or other residues can be added to the mixture according to known data.

As an example of the manner in which the invention is carried out, I will describe the following method of operation, reference being made to the drawing which shows diagrammatically, in front elevation, an apparatus suitable for carrying the invention into practice.

In the drawings, 1 is a suitable steam-heated vessel, adapted to contain crude petroleum.

2 is a second steam-heated vessel, containing water, and 3 is a vessel containing fecula.

4 is a mixer provided with an agitator 5 mounted on a shaft 6 adapted to be ro-

tated by suitable gearing 7 and 8. The mixer is provided with a steam-jacket 9 (shown in dotted lines), steam being admitted through a valve 10 and a pipe 11, 5 while the condensed steam is allowed to escape through a pipe 12 provided with a valve 13.

The vessels 1 and 2 are provided with steam-jackets to which lead the inlet and 10 outlet steam-pipes (not shown) by means of which the petroleum and water may be heated. The vessels are also provided with outlet pipes 14 and 15, respectively, having valves 16 and 17, through which the 15 petroleum and water may be conducted into the mixer 4.

For the manufacture of 100 kgs. of mixture:

(1.) Pour into the mixer 4 10 kilos of 20 flour, (rye-wheat, barley, etc., or other fecula) and set the agitator 5 in motion.

(2.) Let boiling water run on to this flour through pipe 15 and valve 17 until the starch constitutes a mass of the consistence 25 of soft soap. Continue to mix in order that the whole may be perfectly smooth.

(3.) At this moment a small stream of petroleum (heated to 25° to 30° C.) to flow 30 into the mass through pipe 15 and valve 16 in such quantity that it will be absorbed as fast as it arrives.

(4.) Open the steam valve 10 of the mixer so as to heat the paste and cause the grains of fecula to swell. Let a little boiling water (about  $\frac{1}{2}$  liter) run in from time 35 to time.

This operation should be continued in this manner until the quantity of petroleum has arrived at its maximum. For a paste to mix 40 with solid fuel up to the proportion of 25 per cent., about 100 kilos of mixture with 10 kilos of flour and 10 to 15 kilos of water will be obtained; there will therefore be about 75 per cent. of petroleum in the mass.

If a mixture is required to be employed as fuel, it will be necessary at least to double the above stated quantity of flour and add at the end of the operation 10 to 15 per cent. of residues of fatty bodies (stearic, oleic, palmitic, etc.) that is to say, materials which 50 congeal in cooling, as well as 15 to 20 per cent. of coke-dust.

There is no danger of explosion with the products obtained or the agglomerated materials manufactured, by means of this 55 product, the petroleum being really confined in the starchified material.

Having thus described my invention, what I claim is:

1. The improved process for the solidification of a hydrocarbon consisting in causing the grains of a suitable flour or fecula to swell in hot water, and then incorporating a hydrocarbon in said grains, substantially as described. 60

2. The improved process for the solidification of a hydrocarbon consisting in heating water, then mixing with said water a certain quantity of fecula and adding to the mixture a hydrocarbon at a temperature of 70 about 25° to 30° C. substantially as described.

3. An improved process for the solidification of a hydrocarbon consisting of heating separate quantities of water and a hydrocarbon, successively pouring portions of said heated water and hydrocarbon upon the fecula and thoroughly mixing the mass, said heated hydrocarbon and water being poured in varying proportions whereby a more or 75 less thick product is obtained. 80

In testimony whereof I have signed my name to this specification in the presence of two subscribing witnesses.

CHARLES GÉRARD.

Witnesses:

JACQUES SELER,  
CHAS. ROY NASMITH.